

[54] **ELECTROSCOPIC CARRIER PARTICLES HAVING A CARBOXYLIC ACID SURFACE TREATMENT**

[75] Inventor: **John J. Russell, Jr.**, Woodbury, Conn.

[73] Assignee: **Pitney Bowes, Inc.**, Stamford, Conn.

[21] Appl. No.: **920,208**

[22] Filed: **Jun. 28, 1978**

**Related U.S. Application Data**

[63] Continuation-in-part of Ser. No. 811,773, Jun. 30, 1977, abandoned.

[51] Int. Cl.<sup>3</sup> ..... **G03G 13/08; G03G 13/09**

[52] U.S. Cl. ..... **428/403; 428/407**

[58] **Field of Search** ..... **428/403, 404, 407, 402; 427/216; 96/1 S, 1 D, 15 D; 252/62.1 P**

[56] **References Cited**

**U.S. PATENT DOCUMENTS**

**3,922,381** 11/1975 **Datta** ..... **427/216**  
**3,989,648** 11/1976 **Lenhard** ..... **428/403**

|           |         |                |         |
|-----------|---------|----------------|---------|
| 4,063,000 | 12/1977 | Aonuma .....   | 428/403 |
| 4,071,655 | 1/1978  | Brana .....    | 428/403 |
| 4,073,980 | 2/1978  | Westdale ..... | 428/403 |
| 4,113,641 | 9/1978  | Brana .....    | 428/403 |

*Primary Examiner*—Marion McCamish  
*Attorney, Agent, or Firm*—Peter Vrahotes; William D. Soltow, Jr.; Albert W. Scribner

[57] **ABSTRACT**

Disclosed is a treatment of electroscopic carrier particles with a solution of non-halogenated carboxylic acids. Preferably, the carboxylic acid solution is first passed through a dry agent to assure its anhydrous nature. The carrier particles are added to and agitated within the solution a sufficient period to assume complete wetting of the particles. After decanting and filtering, the carrier particles are dried. Carrier particles treated in this manner are less susceptible to oxidation and have particular utility for use in development powders for magnetic brush development units of electrophotography copier equipment.

**3 Claims, No Drawings**

**ELECTROSCOPIC CARRIER PARTICLES  
HAVING A CARBOXYLIC ACID SURFACE  
TREATMENT**

**CROSS-REFERENCE TO RELATED  
APPLICATION**

This is a continuation-in-part of U.S. application Ser. No. 811,773, filed June 30, 1977, and now abandoned.

**BACKGROUND OF THE INVENTION**

With the increased use of plain paper copiers, development powders have enjoyed an increased popularity over liquid toners. Along with the increased use of development powders, magnetic brush units are becoming increasingly popular as opposed to cascading methods. Development powders used with magnetic brush units usually have an iron powder which serves as the carrier material. Inexpensive, untreated iron powders cannot be used in magnetic brush systems since such iron does not have sufficient stability toward rusting and has color and triboelectric charging properties adversely effected by variable humidity conditions. More specifically, the charge to mass ratio (C/M) of the carrier particles will decrease drastically upon exposure to high relative humidity. In order to solve this problem, those in the art have resorted to chemical plating and coating of the iron particles with polymers, oils, waxes and the like and have tried various treatments.

One method described in the literature for the treating of carrier particles is with perfluorinated carboxylic acid. Although this treatment has proven successful, the cost of such materials is relatively high and the number of solvents available for forming treating solutions is limited.

Another problem with prior art developer powders, which are employed in automatic copy machines, is carrier filming problems due to the mechanical rubbing of the carrier surface with the soft toner resins. The gradual accumulation of permanently attached film 40 impairs the normal triboelectric charging of the toner particles in the toner mix. As a result, the toner is either less highly charged or sometimes oppositely charged giving rise to poor copy quality with a high degree of background.

In the literature, several types of plastic coating and electroplating of the carrier have been suggested to overcome the filming problems. Most of the prior art coating methods result in high cost and have other disadvantages such as yielding improper triboelectric charge properties and imparting a very high electrical resistance to the carrier that reduces its development electrode effect and results in poorly filled-in large image areas.

**SUMMARY OF THE INVENTION**

In the art of electrostatographic imaging processing, an electrostatic latent image is formed on a recording surface of a photoconductor. The electrostatic image may then be developed by finely-divided toner particles electrostatically carried by the surface of carrier particles. Preferably, the carrier particles are iron powder or beads.

It has been found that a simple adsorption treatment of iron powder with a carboxylic acid solution produces a treated iron which has good stability to rusting under high relative humidity, a constant triboelectric charge property under all conditions when mixed with stan-

dard toners, low dusting of the toner in a magnetic brush unit and the treatment allows the use of lower biased voltage during development which improves the reliability of machine performance.

- 5 By using the treated carrier particles of this invention, an improved electrophotographic process is obtained. In this improved process, a latent electrostatic image is contacted with a developer mixture including the treated carrier particles of this invention. Additionally, the process yields an inexpensive way of treating carrier particles and the process may be carried out with a wide selection of solvents.

**DESCRIPTION OF THE PREFERRED  
EMBODIMENT**

15 The core of the carrier particle formed by the present invention may be any material which can react chemically with the carboxylic acid compounds of this invention. Thus, by way of example, the material of the core 20 of the carrier particle may be sand, glass beads, metallic beads or metallic powders. As used in this specification, including the appended claims, the term metal and metallic is intended to include elemental metals as well as their oxides, carbides and other forms of metallic compounds and alloys which have a solid form.

25 The core of carrier particles of the preferred embodiment is a ferromagnetic material such as iron or steel. Other suitable ferromagnetic materials such as magnetic oxides and alloys of copper-nickel-iron, for example, also may be employed. The size of the core may be between 40 and 1000 microns with the preferred size range being between 50 and 400 microns.

30 The carboxylic acid may be selected from a number of classes including aliphatic, branched and unbranched, substituted and unsubstituted, and aromatic, substituted and unsubstituted.

35 In the use of such carboxylic acids it has been found preferable to assure the anhydrous nature of such acids. This is accomplished by passing the carboxylic acid through a drying agent such as a desiccant or molecular sieve immediately prior to use.

40 Examples of suitable carboxylic acids are as follows:

**ALIPHATIC CARBOXYLIC ACIDS**

- 45 4-acetamidobutyric acid  
acetic acid, glacial  
11,3-acetonedicarboxylic acid  
4-acetylbutyric acid  
50 acetylenedicarboxylic acid  
N-acetylmuramic acid  
aconitic acid  
acrylic acid  
1-adamantaneacetic acid  
55 1,3-adamantanediacetic acid  
adipic acid  
adipic acid monoethyl ester  
adipic acid monomethyl ester  
 $\beta$ -alanine  
60 DL-2-amino adipic acid  
3-aminobutyric acid  
4-aminobutyric acid  
6-aminocaproic acid  
12-aminododecanoic acid  
65 DL-3-amino-3-hydroxybutyric acid  
pp-aminophenylacetic acid  
3-amino-3-phenylpropionic acid  
11-aminoundecanoic acid

5-aminovaleric acid  
 azelaic acid  
 azelaic acid monomethyl ester  
 4,4'-azobis-(4-cyanovaleric acid)  
 5-benzamidovaleric acid  
 Benzilic acid  
 1,4-benzodioxan-6-acetic acid  
 4-benzoylbutyric acid  
 benzoylformic acid  
 3-benzoylpropionic acid  
 5-benzylvaleric acid  
 benzylmalonic acid

#### ALIPHATIC CARBOXYLIC ACIDS

5-benzyloxyindole-3-acetic acid  
 S-benzylthioglycolic-acid  
 2,2-Bis-(hydroxymethyl)-propionic acid  
 tert.-butylacetic acid  
 n-butyric acid  
 cacotheine  
 N-carbobenzoyloxy-L-aspartic acid  
 cholesteryl hydrogen succinate  
 cholic acid  
 cinnamylidenemalonic acid  
 citraconic acid  
 citric acid  
 crotonic acid  
 cyanoacetic acid  
 cyclohexanebutyric acid  
 1,1-cyclohexanediacetic acid  
 cyclohexanepropionic acid  
 cyclohexylacetic acid  
 cyclohexyphenylacetic acid  
 cyclohexylphenylglycolic acid  
 2-cyclohexene-1-acetic acid  
 cyclopentylacetic acid  
 3-cyclopentylpropionic acid  
 1,10-decanedicarboxylic acid  
 decanoic acid  
 decanoic acid  
 deoxycholic acid  
 diglycolic acid  
 2,5-dihydroxy-p-benzenediacetic acid  
 3,4-dihydroxyhydrocinnamic acid  
 dihydroxymaleic acid  
 DL-3,4-dihydroxymandelic acid  
 3,4-dihydroxyphenylacetic acid  
 dihydroxytartaric acid  
 (2,5-dimethoxyphenyl)-acetic acid  
 (3,4-dimethoxyphenyl)-acetic acid  
 3-(3,4-dimethoxyphenyl)-propionic acid  
 3,3-dimethylacrylic acid  
 3,3-dimethylglutaric acid  
 dimethylmalonic acid  
 2,2-dimethylsuccinic acid  
 diphenylacetic acid  
 2,2-diphenylpropionic acid  
 3,3-diphenylpropionic acid  
 meso-2,3-diphenylsuccinic acid  
 dithiodiglycolic acid  
 3,3'-dithiodipropionic acid  
 di-p-toluoyl-d-tartaric acid  
 di-p-tolyacetic acid  
 1,12-dodecanedicarboxylic acid  
 eicosanoic acid  
 elaidic acid  
 erucic acid  
 ethyxyacetic acid

4-ethoxy-3-methoxyphenylacetic acid

#### ALIPHATIC CARBOXYLIC ACIDS

p-ethoxyphenylacetic acid  
 5 3-ethoxypropionic acid  
 3-ethoxypropionic acid  
 2-ethylhexanoic acid  
 2-ethyl-2-hydroxybutyric acid  
 5-ethyl-3-indoleacetic acid  
 10 ethylmalonic acid  
 2-ethyl-2-methylsuccinic acid  
 formic acid  
 o-formylphenoxyacetic acid  
 fumaric acid  
 15 fumaric acid monoethyl ester  
 furylacrylic acid  
 gluconic acid  
 glutaconic acid  
 glutaric acid  
 20 glyceric acid  
 glycolic acid  
 n-heptadecanoic acid  
 heptanoic acid  
 hexadecanedioic acid  
 25 2,4-hexadienoic acid  
 hexanoic acid  
 hexanoic acid  
 homophthalic acid  
 homovanillic acid  
 30 5-hydantoinacetic acid  
 hydrocinnamic acid  
 trans- $\beta$ -hydromuconic acid  
 33-hydroxybutyric acid  
 16-hydroxyhexadecanoic acid  
 35 5-hydroxyindole-3-acetic acid  
 2-hydroxyisobutyric acid  
 2-hydroxyisobutyric acid  
 m-hydroxymandelic acid  
 2-hydroxy-2-methylbutyric acid  
 40 o-hydroxyphenylacetic acid  
 m-hydroxyphenylacetic acid  
 p-hydroxyphenylacetic acid  
 3-(p-hydroxyphenyl)-propionic acid  
 p-hydroxyphenylpyruvic acid  
 45 3-hydroxypropionic acid  
 indole-3-acetic acid  
 3-indoleacrylic acid  
 3-indolebutyric acid  
 DL- $\beta$ -3-indolelactic acid  
 50 indole-3-pyruvic acid  
 isobutyric acid  
 itaconic acid  
 2-ketobutyric acid  
 2-ketoglutaric acid  
 55 ketomalonic acid monohydrate  
 4-ketopimelic acid  
 DL-lactic acid  
 DL-lactic acid

60 ALIPHATIC CARBOXYLIC ACIDS

L-(+)-lactic acid  
 lauric acid  
 levulinic acid  
 linolenic acid  
 65 maleic acid  
 dd-malic acid  
 DL-malic acid  
 1-malic acid

malonic acid  
 d-mandelic acid  
 DL-mandelic acid  
 11-mandelic acid  
 1-menthoxyacetic acid  
 mercaptoacetic acid  
 3-mercaptopropionic acid  
 mercaptosuccinic acid  
 mesaconic acid  
 methacrylic acid  
 3-(p-methoxybenzoyl)-propionic acid  
 5-methoxyindole-3-acetic acid  
 5-methoxy-2-methyl-3-indoleacetic acid  
 3-methoxyphenylacetic acid  
 4-methoxyphenylacetic acid  
 4-(p-methoxyphenyl)-butyric acid  
 3-(o-methoxyphenyl)-propionic acid  
 3-(o-methoxyphenyl)-propionic acid  
 (+)-3-methyladipic acid  
 3-methyladipic acid  
 methylaminomethyltartronic acid  
 3,4-methylenedioxycinnamic acid  
 mono-methyl glutarateetic acid  
 2-methylglutaric acid  
 3-methylglutaric acid  
 methylmalonic acid  
 mono-methyl succinate  
 methylsuccinic acid  
 $\beta$ -methyltricarballylic acid  
 mucic acid  
 trans,trans-muconic acid  
 muramic acid  
 myristic acid  
 myristic acid  
 (2-naphthoxy)-acetic acid  
 1-naphthylacetic acid  
 2-naphthyla  
 cetic acid  
 3,3',3''-nitrilotripropionic acid  
 o-nitrophenylacetic acid  
 m-nitrophenylacetic acid  
 p-nitrophenylacetic acid

## ALIPHATIC CARBOXYLIC ACIDS

4-(p-nitrophenyl)-butyric acid  
 o-nitrophenylpyruvic acid  
 3-nitropropionic acid  
 nonanoic acid  
 2-norbornaneacetic acid  
 5-norbornene-2-acrylic acid  
 octanoic acid  
 octanoic acid  
 trans-2-octenoic acid  
 oxalacetic acid  
 oxamic acid  
 palmitic acid  
 n-pentadecanoic acid  
 phenoxyacetic acid  
 2-phenoxybutyric acid  
 3-phenoxypropionic acid  
 11-phenoxyundecanoic acid  
 phenylacetic acid  
 2-phenylbutyric acid  
 3-phenylbutyric acid  
 4-phenylbutyric acid  
 o-phenylenediacetic acid  
 m-phenylenediacetic acid  
 p-phenylenedipropionic acid

L-(--)-3-phenylactic acid  
 phenylmalonic acid  
 phenylpropionic acid  
 2-phenylpropionic acid  
 5-phenyl-2-pyrrolepropionic acid  
 phenylsuccinic acid  
 5-phenylvaleric acid  
 pimelic acid  
 cis-pinonic acid  
 10 propionic acid  
 propionic acid  
 2-pyridylacetic acid hydrochloride  
 3-pyridylacetic acid hydrochloride  
 $\beta$ -(3-Pyridyl)-acetic acid  
 15 pyruvic acid  
 sebamic acid  
 stearic acid  
 styrilacetic acid  
 suberic acid  
 20 succinamic acid  
 succinic acid  
 d-tartaric acid  
 DL-tartaric acid hydrate  
 l-tartaric acid  
 25 meso-tartaric acid hydrate  
 tartaric acid  
 3-3-tetramethyleneglutaric acid  
 4-thianaphtheneacetic acid  
 3-(2-thienyl)-acrylic acid  
 30 4-(2-thienyl)-butyric acid

## ALIPHATIC CARBOXYLIC ACIDS

S-(thiobenzoyl)-thioglycolic acid  
 DL-thioctic acid  
 35 thioglycolic acid  
 3,3'-thiodipropionic acid  
 thiolactic acid  
 thiophenoxyacetic acid  
 tiglic acid  
 40 o-tolylacetic acid  
 m-tolylacetic acid  
 p-tolylacetic acid  
 triacontanoic acid  
 tricarballylic acid  
 45 n-tridecanoic acid  
 3,4,5-trimethoxyphenylacetic acid  
 trimethylacetic acid  
 triphenylacetic acid  
 tropic acid  
 50 1,11-undecanedicarboxylic acid  
 undecandieic acid  
 undecanoic acid  
 undecylenic acid  
 valeric acid  
 55 vinylacetic acid

## CINNAMIC ACIDS

p-acetamidocinnamic acid  
 p-aminocinnamic acid hydrochloride  
 60 2,3-Bis-(p-methoxyphenyl)-acrylic acid  
 o-carboxycinnamic acid  
 trans-cinnamic acid  
 $\alpha$ -cyano-3-hydroxycinnamic acid  
 2,4-dichlorocinnamic acid  
 65 2,6-dichlorocinnamic acid  
 3,4-dichlorocinnamic acid  
 3,4-dihydroxycinnamic acid  
 2,4-dimethoxycinnamic acid

2,5-dimethoxycinnamic acid  
 3,4-dimethoxycinnamic acid  
 3,5-dimethoxycinnamic acid  
 3,5-dimethoxy-4-hydroxycinnamic acid  
 4-ethoxy-3-methoxycinnamic acid  
 p-formylcinnamic acid  
 o-hydroxycinnamic acid  
 m-hydroxycinnamic acid  
 cis-p-hydroxycinnamic acid  
 p-hydroxycinnamic acid  
 3-hydroxy-4-methoxycinnamic acid  
 4-hydroxy-3-methoxycinnamic acid  
 o-methoxycinnamic acid  
 m-methoxycinnamic acid  
 p-methoxycinnamic acid  
 $\alpha$ -methylcinnamic acid  
 p-methylcinnamic acid  
 o-nitrocinnamic acid

## CINNAMIC ACIDS

m-nitrocinnamic acid  
 p-nitrocinnamic acid  
 $\alpha$ -phenylcinnamic acid  
 m-phenylenediacrylic acid  
 p-phenylenediacrylic acid  
 2,4,5-trimethoxycinnamic acid  
 3,4,5-trimethoxycinnamic acid

## AROMATIC CARBOXYLIC ACIDS

p-acetamidobenzoic acid  
 N-acetylanthranilic acid  
 2-acetylbenzoic acid  
 4-acetylbenzoic acid  
 acetylsalicylic acid  
 m-aminobenzoic acid  
 p-aminobenzoic acid  
 4-amino-3,5-dimethylbenzoic acid  
 5-aminosophthalic acid  
 2-amino-3-methylbenzoic acid  
 2-amino-4-methylbenzoic acid  
 2-amino-5-methylbenzoic acid  
 3-amino-4-methylbenzoic acid  
 4-amino-3-methylbenzoic acid  
 3-amino-2-naphthoic acid  
 5-amino-2-nitrobenzoic acid  
 3-amino-5-nitrosalicylic acid monohydrate  
 4-aminosalicylic acid  
 5-aminosalicylic acid  
 4-aminosulfonyl-1-hydroxy-2-naphthoic acid  
 o-anisic acid  
 m-anisic acid  
 p-anisic acid  
 anthracene-9-carboxylic acid  
 anthranilic acid  
 o-antraniloylbenzoic acid  
 aristolochic acid  
 aurintricarboxylic acid  
 1,2,4,5-benzenetetracarboxylic acid  
 1,2,4-benzenetricarboxylic acid  
 1,3,5-benzenetricarboxylic acid  
 benzoic acid  
 2-benzoylbenzoic acid  
 4-benzoylbenzoic acid  
 2-bibenzylcarboxylic acid  
 2-biphenylcarboxylic acid  
 4-biphenylcarboxylic acid  
 4-n-butoxybenzoic acid  
 p-tert-butylbenzoic acid

3-tert-butyl-5-methylsalicylic acid  
 2-carboxybenzaldehyde  
 4-carboxybenzaldehyde  
 p-carboxybenzenesulfonamide  
 5 o-carboxycinnamic acid  
 2'-carboxy-2-hydroxybenzophenone

## AROMATIC CARBOXYLIC ACIDS

cholesteryl hydrogen phthalate  
 10 3-cyanobenzoic acid  
 4-cyanobenzoic acid  
 p-2-cyclohexenylbenzoic acid  
 3,4-diaminobenzoic acid  
 3,5-diaminobenzoic acid  
 15 3,5-diaminobenzoic acid hydrochloride  
 3,5-Di-tert-butyl-2,6-dihydroxybenzoic acid  
 3,5-Di-tert-butyl-4-hydroxybenzoic acid  
 4-diethylaminosalicylic acid  
 2,3-dihydroxybenzoic acid  
 20 2,4-dihydroxybenzoic acid  
 2,5-dihydroxybenzoic acid  
 2,6-dihydroxybenzoic acid  
 3,4-dihydroxybenzoic acid  
 3,5-dihydroxybenzoic acid  
 25 3,5-dilisopropylsalicylic acid  
 2,3-dimethoxybenzoic acid  
 2,4-dimethoxybenzoic acid  
 2,6-dimethoxybenzoic acid  
 3,4-dimethoxybenzoic acid  
 30 3,5-dimethoxybenzoic acid  
 3-dimethylaminobenzoic acid  
 4-dimethylaminobenzoic acid  
 4-dimethylaminosalicylic acid  
 2,4-dimethylbenzoic acid  
 35 2,5-dimethylbenzoic acid  
 2,6-dimethylbenzoic acid  
 3,4-dimethylbenzoic acid  
 3,5-dimethylbenzoic acid  
 2,6-nitrobenzoic acid  
 40 3,4-dinitrobenzoic acid  
 3,5-dinitrobenzoic acid  
 diphenic acid  
 5,5'-dithiobis-(2-nitrobenzoic acid)  
 2,2'-dithiosalicylic acid  
 45 p-dodecyloxybenzoic acid  
 p-ethoxybenzoic acid  
 flufenamic acid  
 1-fluorenecarboxylic acid  
 9-fluorenone-2-carboxylic acid  
 50 9-fluorenone-4-carboxylic acid  
 5-formylsalicylic acid  
 o-(hexadecylthio)-benzoic acid  
 homophthalic acid  
 m-hydroxybenzoic acid  
 55 p-hydroxybenzoic acid  
 2-(p-hydroxybenzoyl)-benzoic acid  
 4-hydroxy-3-methoxybenzoic acid  
 3-hydroxy-4-methylbenzoic acid  
 3-hydroxy-4-methyl-2-nitrobenzoic acid  
 60 1-hydroxy-2-naphthoic acid  
 3-hydroxy-2-naphthoic acid  
 3-hydroxy-4-nitrobenzoic acid  
 8-hydroxyquinoline-7-carboxylic acid

## AROMATIC CARBOXYLIC ACIDS

65 indole-5-carboxylic acid  
 isophthalic acid  
 metallitic trianhydride

3-methoxy-3-methylbenzoic acid  
 3-methoxy-2-nitrobenzoic acid  
 3-methoxy-4-nitrobenzoic acid  
 5-methoxysalicylic acid  
 p-(methylamino)-benzoic acid  
 N-methylanthranilic acid  
 2-methyl-3-nitrobenzoic acid  
 2-methyl-6-nitrobenzoic acid  
 3-methyl-2-nitrobenzoic acid  
 3-methyl-4-nitrobenzoic acid  
 3-methyl-6-nitrobenzoic acid  
 4-methyl-3-nitrobenzoic acid  
 3-methylsalicylic acid  
 5-methylsalicylic acid  
 p-(methylsulfonyl)-benzoic acid  
 4-methylsulfonyl-3-nitrobenzoic acid  
 p-(methylthio)-benzoic acid  
 4-methylthio-3-nitrobenzoic acid  
 5-(methylthio)-salicylic acid  
 2,3-naphthalenedicarboxylic acid  
 1-naphthoic acid  
 2-naphthoic acid  
 4-nitroanthranilic acid  
 o-nitrobenzoic acid  
 m-nitrobenzoic acid  
 p-nitrobenzoic acid  
 5-nitroisophthalic acid  
 p-nitroperoxybenzoic acid  
 3-nitrophthalic acid  
 4-nitrophthalic acid  
 nitroterephthalic acid  
 5-tert-octylsalicylic acid  
 3,4,9,10-perylenetetracarboxylic dianhydride  
 oo-henoxybenzoic acid  
 N-phenylanthranilic acid  
 $\alpha$ -phenyl-o-toluic acid  
 phthalic acid  
 o-phthalimidobenzoic acid  
 pieronylic acid  
 potassium hydrogen phthalate  
 salicylic acid  
 4,4'-sulfonyldibenzoinic acid  
 syringic acid  
 terephthalic acid  
 tetramethylterephthalic acid  
 thiosalicylic acid  
 o-toluic acid  
 m-toluic acid  
 p-toluic acid  
 2,4,5-trimethoxybenzoic acid  
 2,4,6-trimethoxybenzoic acid  
 3,4,5-trimethoxybenzoic acid  
 2,4,6-trimethylbenzoic acid

## ALICYCLIC CARBOXYLIC ACIDS

1-adamantanecarboxylic acid  
 trans-4-(aminomethyl)-cyclohexanecarboxylic acid  
 betulinic acid  
 di-3-camphorcarboxylic acid  
 d-camphoric acid  
 cyclobutanecarboxylic acid  
 1,1-cyclobutanedicarboxylic acid  
 trans-1,2-cyclobutanedicarboxylic acid  
 cycloheptanecarboxylic acid  
 4-cycloheptene-1-carboxylic acid  
 cyclohexanecarboxylic acid  
 cis-1,2-cyclohexanedicarboxylic acid  
 trans-1,2-cyclohexanedicarboxylic acid

trans-1,4-cyclohexanedicarboxylic acid  
 4-cyclooctene-1-carboxylic acid  
 cyclopentanecarboxylic acid  
 cis,cis,cis-1,2,3,4-cyclopentane-tetracarboxylic acid  
 5-cyclopropanecarboxylic acid  
 9-fluorenecarboxylic acid  
 gibberellic acid  
 $\beta$ -glycyrrhetic acid  
 hexahydro-4-methylphthalic acid  
 10 1-hydroxycycloheptanecarboxylic acid  
 9-hydroxy-9-fluorenecarboxylic acid  
 1-(p-methoxyphenyl)-1-cyclohexane-carboxylic acid  
 1-(p-methoxyphenyl)-1-cyclopentane-carboxylic acid  
 1-(p-methoxyphenyl)-1-cyclopropane-carboxylic acid  
 15 1-methyl-1-cyclohexanecarboxylic acid  
 1-methylindene-2-carboxylic acid  
 1-phenyl-1-cyclohexanecarboxylic acid  
 1-phenylcyclopentanecarboxylic acid  
 1-phenyl-1-cyclopropanecarboxylic acid  
 20 trans-2-phenylcyclopropanecarboxylic acid  
 quinic acid  
 shikimic acid  
 1-(p-tolyl)-1-cyclohexanecarboxylic acid  
 1-(p-tolyl)-1-cyclopentanecarboxylic acid  
 25 1-(p-tolyl)-1-cyclopropanecarboxylic acid

## OTHER CARBOXYLIC ACIDS

N-acetylneurameric acid  
 alginic acid  
 30 2-aminonicotinic acid  
 6-aminopenicillanic acid  
 3-aminopyrazole-4-carboxylic acid  
 1-benzylindole-3-carboxylic acid  
 cinnoline-4-carboxylic acid  
 35 citrazinic acid  
 coumaric acid monohydrate  
 coumarin-3-carboxylic acid  
 diethylstilbestrol monoglucuronide  
 4,8-dihydroxyuinoline-2-carboxylic acid  
 40 2,3,4,6-di-O-isopropylidene-2-keto-L-gulonic acid  
 monohydrate

## OTHER CARBOXYLIC ACIDS

6,6'-dithiodinicotinic acid  
 45 5-ethyl-2-indolecarboxylic acid  
 ferrocenecarboxylic acid  
 1,1'-ferrocenedicarboxylic acid  
 3,4-furandicarboxylic acid  
 2-furoic acid  
 50 3-furoic acid  
 hyalueronic acid  
 5-hydroxy-2-indolecarboxylic acid  
 4-hydroxy-7-methyl-1,8-naphthyridine-3-carboxylic acid  
 55 2-hydroxy-6-methylpyridine-3-carboxylic acid  
 6-hydroxynicotinic acid  
 4-hydroxy-6-nitro-3-quinoliniccarboxylic acid  
 3-hydroxypicolinic acid  
 4-hydroxyquinoline-2-carboxylic acid  
 60 3-hydroxy-2-quinoxalinecarboxylic acid  
 indole-2-carboxylic acid  
 DL-isocitric acid lactone  
 isodehydracetic acid  
 isonicotinic acid  
 65 isonipecotic acid  
 1-isoquinolinecarboxylic acid  
 5-methoxyindole-2-carboxylic acid  
 1-methylindole-2-carboxylic acid

5-methylindole-2-carboxylic acid  
 1-methyl-5-oxo-3-pyrrolidinocarboxylic acid  
 5-methyl-3-phenylisoxazole-4-carboxylic acid  
 N-methylpyrrole-2-carboxylic acid  
 5-methyl-2-thiophenecarboxylic acid  
 nalidixic acid  
 nicotinic acid  
 nicotinic acid N-oxide  
 5-nitro-2-furoic acid  
 picolinic acid  
 picolinic acid N-oxide pipocolinic acid  
 2-piperidinocinchoninic acid  
 2-pyrazinecarboxylic acid  
 2,3-pyrazinedicarboxylic acid  
 3,5-pyrazoledicarboxylic acid  
 2,6-pyridinedicarboxylic acid  
 3,4-pyridinedicarboxylic acid  
 3,5-pyridinedicarboxylic acid  
 pyrrole-2-carboxylic acid  
 L-2-pyrrolidone-5-carboxylic acid  
 quinaldic acid  
 3-quinolonecarboxylic acid  
 tetrahydrofuran-2,3,5-tetracarboxylic acid  
 L-thiazolidine-4-carboxylic acid  
 2-thiophenecarboxylic acid  
 xanthene-9-carboxylic acid

A number of solvents may be used for preparing the carboxylic acid solution including 1,1,2 trichloro 1,2,2 trifluoroethane, chloroform, tetrahydrofuran, methanol and methyl ethyl ketone. The concentration of the carboxylic acid solution should be such that the treatment of the carrier particle would provide a monomolecular about the surface thereof. This is preferable since the adherence of the molecules upon the carrier particle is by adhesion and any excess would tend to be dete- 30  
 rimented as the excess would easily be separated and tend to contaminate the development powder. To obtain a monomolecular, the concentration would be a function of the surface area to be covered, the molecular weight of the carboxylic acid as well as the molecular dimension of the acid. It has been found that a concentration of 0.001 to 0.030 grams of acid to 100 grams of iron powder has been a satisfactory range for the material disclosed herein. It will be understood, however, that this range is not all encompassing as the concentration 45  
 may fall below or above this satisfactory range depending upon the acid selected.

The amount of acid required may be calculated in accordance with the following illustration using stearic acid.

The surface area of the iron powder was measured by BET and was found to be  $0.05054 \text{ m}^2/\text{gm} = 0.05054 \text{ m}^2/\text{gm} \times 10^4 \text{ cm}^2/\text{m}^2 = 505.4 \text{ cm}^2/\text{gm}$ .

The area covered by a single molecule of fatty acid is equal to  $21 \times 10^{-16} \text{ sq cm}/\text{molecule}$ .

Therefore  $505.4 \text{ cm}^2/\text{gm iron} / 21 \times 10^{-16} \text{ cm}^2/\text{molecule} = 24.07 \times 10^{16} \text{ molecule/gm iron}$ .

Since there are  $6.02 \times 10^{23}$  (Avogadro's number) molecules per mole of any substance then  $24.07 \times 10^{16} \text{ molecules/gm iron} / 6.02 \times 10^{23} \text{ molecules/- 60 mole} = 4 \times 10^{-7} \text{ moles acid/gm iron}$ .

For stearic acid whose molecular weight is 284.5 one would need  $4 \times 10^{-7} \text{ moles acid} \times 100 \text{ gms iron} \times 284.5 = 0.011380 \text{ gms}$ .

A number of commercial toners were used with the 65 carrier particle treated in accordance with the instant invention and it was found that the treated particle served well with any of these toners. Consequently it

does not appear that the selection of toner is important relative to the treated carrier particle.

#### EXAMPLE I

5 Five hundred grams of iron powder was added to a solution of 0.075 g of myristic acid dissolved in 100 mls. of 1,1,2 trichloro 1,2,2 trifluoroethane. This mixture was then stirred at room temperature until the solvent was completely evaporated. A development powder was 10 then prepared using 97.6 gms. of thusly treated iron and 2.4 gms. of toner made from an epoxy base resin modified with polyvinyltoluene. The resulting charge to mass ratio (C/M) was  $5.7 \mu\text{C}/\text{gm}$ .

15

#### EXAMPLE II

Iron powder was treated as in Example I except that the solvent was evaporated in an oven at 70 degrees C. A developer was prepared as previously described and the resulting C/M was  $10.3 \mu\text{C}/\text{gm}$ .

20

#### EXAMPLE III-XVI

The acids listed in Table I were used to treat iron as described in Example I, the solution in each case having a concentration of 0.015 gms/100 gms. iron. Development powders were then prepared as described in Example II using the following toners:

Toner U—The toner of Examples I and II.

Toner V—A styrene acrylic copolymer described in Example IV of U.S. Pat. No. 3,980,576.

Toner W—A polyester resin described in U.S. Pat. No. 3,681,106 and available from Xerox Corporation under the Trademark 3100 DRY INK.

Table I shows the C/M obtained using various toners with the acids from Table I.

TABLE I

| acid<br>Number | Acid<br>Trivial<br>Name        | Acid<br>Formula                                                              |
|----------------|--------------------------------|------------------------------------------------------------------------------|
| 9              | 2 ethylhexanoic                | $\text{CH}_3(\text{CH}_2)_4\text{CH}(\text{C}_2\text{H}_5)\text{COOH}$       |
| 2              | palmitic                       | $\text{CH}_3(\text{CH}_2)_{14}\text{COOH}$                                   |
| 1              | myristic                       | $\text{CH}_3(\text{CH}_2)_{12}\text{COOH}$                                   |
| 3              | stearic                        | $\text{CH}_3(\text{CH}_2)_{16}\text{COOH}$                                   |
| 4              | oxalic                         | $\text{HOOCCOOH}$                                                            |
| 5              | citric                         | $\text{HO}(\text{COOH})\text{CH}_2\text{COOH}_2$                             |
| 6              | tannic                         | $\text{C}_7\text{H}_5\text{O}_6$                                             |
| 7              | tartaric                       | $\text{HOOC}(\text{CHOH})_2\text{COOH}$                                      |
| 8              | ethylenediamine<br>tetraacetic | $(\text{HOOCCH}_2)_2\text{N}(\text{CH}_2)\text{N}(\text{CH}_2\text{COOH})_2$ |
| 10             | benzoic                        | $\text{C}_6\text{H}_5\text{COOH}$                                            |
| 11             | phthalic                       | $1,2\text{-C}_6\text{H}_4(\text{COOH})_2$                                    |
| 12             | salicylic                      | $2\text{-HO}C_6H_4\text{COOH}$                                               |
| 13             | gallic                         | $3,4,5\text{-}(\text{HO})_3\text{C}_6\text{H}_2\text{COOH}$                  |
| 14             | p-nitrobenzoic                 | $4\text{-O}_2\text{NC}_6\text{H}_4\text{COOH}$                               |
| 15             | phenoxyacetic                  | $\text{C}_6\text{H}_5\text{OCH}_2\text{COOH}$                                |

TABLE II

| Acid | Cone.<br>g/100g iron | C/M @ 20% RH micro<br>coulombs/gram toner |        |        |
|------|----------------------|-------------------------------------------|--------|--------|
|      |                      | U                                         | V      | W      |
| .2   | 0.015                | + 16.3                                    | + 12.9 | - 15.9 |
| .3   | 0.015                | + 17.6                                    | + 17.9 | - 15.1 |
| .4   | 0.015                | + 13.7                                    |        |        |
| .5   | 0.006                | + 16.0                                    |        |        |
| .6   | 0.015                | + 14.1                                    |        |        |
| .7   | 0.008                | + 12.4                                    |        |        |
| .8   | 0.004                | + 8.5                                     |        |        |
| .9   | 0.015                | + 25.5                                    | + 17.8 | - 12.7 |
| 10   | 0.015                | + 12.2                                    | + 6.9  | 21.4   |
| 11   | 0.006                | + 9.3                                     |        |        |
| 12   | 0.008                | + 11.1                                    |        |        |
| 13   | 0.006                | + 12.9                                    |        |        |

TABLE II-continued

| Acid | Conc.<br>g/100g iron | C/M @ 20% RH micro<br>coulombs/gram toner |   |   |
|------|----------------------|-------------------------------------------|---|---|
|      |                      | U                                         | V | W |
| 14   | 0.015                | +21.7                                     |   |   |
| 15   | 0.015                | + 8.9                                     |   |   |

TABLE III shows the C/M obtained using toner U and varying the acid concentration (gm/acid/100 gm iron).

TABLE III

| Acid                | C/M<br>iron treated            |       | C/M<br>iron |       |       |      |
|---------------------|--------------------------------|-------|-------------|-------|-------|------|
|                     | C/M<br>w/Freon TA<br>& no acid | 0.004 | 0.008       | 0.015 | 0.030 |      |
| 2-ethyl<br>hexanoic | 15.6                           | 15.6  | 29.0        | 27.5  | 21.4  | 24.0 |
| stearic             | 15.6                           | 15.6  | 18.9        | 11.9  | 17.6  | 6.7  |

The following data indicates the advantage of maintaining anhydrous conditions.

A molecular sieve (Davison Chemical Co., Baltimore, Maryland, Grade 574,) having an effective pore size of 4 A°, and an 8-12 mesh, was added to 20 ml of Freon TA, a solvent commercially available from DuPont Corp. of 89 W/O 1,1,2 trichloro 1,2,2 trichloroethane and 11 w/O acetone containing 0.005 gm 2 ethyl hexanoic acid. The solutions were then used to treat 100 grams of iron powder and the results obtained are shown in Table IV.

TABLE IV

| 5        | Freon TA<br>having |                  |                              |                |                |                |
|----------|--------------------|------------------|------------------------------|----------------|----------------|----------------|
|          | Untreated          | Freon<br>No Acid | 2 ethyl hexanoic<br>No Sieve | 0.5gm<br>Sieve | 1.0gm<br>Sieve | 2.0gm<br>Sieve |
| C/M 13.0 | 13.2               |                  | 10.2                         | 17.4           | 19.4           | 16.1           |

The following results show the protective action against oxidation after samples were exposed to 90 degrees F. and 85% relative humidity for one week.

The reflectance was determined with a Hunter Lab color/difference Meter D-25D2.

| 15                                                             | initial<br>reflectivity     | reflectivity after<br>1 week |                    |
|----------------------------------------------------------------|-----------------------------|------------------------------|--------------------|
|                                                                |                             | L + + 40.4 a - 0.5, b + 1.7  | + 38.9 - 0.7 + 2.1 |
| untreated                                                      | L + + 40.4 a - 0.5, b + 1.7 | + 38.9 - 0.7 + 2.1           |                    |
| treated with<br>0.015g 2-ethyl<br>hexanoic acid<br>100g of non | L + + 38.9 a - 0.6, b + 1.8 | + 39.3 - 0.7 + 1.9           |                    |

What is claimed is:

1. A carrier for use in a magnetic brush development unit for the electrophotographic development of latent electro-static images consisting of ferromagnetic particles having adhered to the surface thereof a monomolecular layer of a non-halogenated carboxylic acid.
2. The carrier of claim 1 wherein said carboxylic acid is selected from the group consisting of aliphatic carboxylic acid, cinnamic acids, aromatic carboxylic acid and alicyclic.
3. The carrier particle of claim 1 wherein said carrier particle is iron.

\* \* \* \* \*

35

40

45

50

55

60

65